

**United States Patent** [19]

Schmalz

[11] **Patent Number:** 4,938,832[45] **Date of Patent:** Jul. 3, 1990

[54] **CARDABLE HYDROPHOBIC POLYPROPYLENE FIBER, MATERIAL AND METHOD FOR PREPARATION THEREOF**

[75] **Inventor:** A. Chandler Schmalz, Conyers, Ga.

[73] **Assignee:** Hercules Incorporated, Wilmington, Del.

[21] **Appl. No.:** 358,985

[22] **Filed:** May 30, 1989

[51] **Int. Cl.<sup>5</sup>** ..... B05D 3/02

[52] **U.S. Cl.** ..... 156/308.8; 156/296; 156/305; 427/393.1; 428/290; 524/274

[58] **Field of Search** ..... 156/296, 305, 308.2, 156/308.6, 308.8; 524/274; 427/393.1; 428/290

[56]

**References Cited****U.S. PATENT DOCUMENTS**

3,341,451 9/1967 Duziuba et al. ..... 252/8.6  
3,423,314 1/1969 Campbell ..... 427/393.1 X  
3,926,816 12/1975 Cohen et al. ..... 252/8.9  
4,143,206 3/1979 Jäger ..... 427/393.1 X  
4,535,013 8/1985 Kuhn ..... 156/308.2 X  
4,705,704 11/1987 Lane et al. ..... 427/393.1 X

*Primary Examiner*—Robert L. Lindsay  
*Attorney, Agent, or Firm*—John E. Crowe

[57]

**ABSTRACT**

A method for placing hydrophobic polyolefin fiber in condition for cutting, carding and production of non-woven material without substantial sacrifice in desired hydrophobic properties in the corresponding nonwoven, by utilization of a sequential treatment of the fiber with a neutralized phosphoric acid ester and a polysiloxane of defined classes.

19 Claims, No Drawings

**CARDABLE HYDROPHOBIC POLYPROPYLENE  
FIBER, MATERIAL AND METHOD FOR  
PREPARATION THEREOF**

The present invention relates to a method utilizing 10 topically applied modifier compositions arranged in sequence and in a unique arrangement whereby polyolefin containing hydrophobic fiber or filament is made receptive to interim cutting and carding operations without loss of hydrophobicity in the resulting fiber or nonwoven product.

**BACKGROUND**

While the manufacture of polyolefin based fiber, webs and corresponding nonwoven materials are well known in the textile art, attempts to broadly apply such knowledge to produce products in the area of personal hygiene, such as catamenial devices, disposable diapers, 20 incontinence pads and the like, have met with serious technical problems.

In general, such products must have a fluid absorbent core, usually comprising one or more layers of absorbent material such as wood pulp, rayon, gauze, tissue 25 and the like and, in some cases, synthetic hydrophilic material such as a hydrophilic polyurethane foam.

Such fluid absorbing core is most generally fabricated in the form of a thermally bonded pad, of wood pulp, fiber and conjugate fiber, having a rectangular or somewhat oval shape. To protect a wearer's clothing, and surrounding areas from stain or wetting by fluids already absorbed in such a core, a fluid-impervious barrier sheet is usually required. In general, the absorbent 30 device is positioned against the body of the user with hydrophilic material facing and contacting the body and the fluid impervious barrier sheet positioned on the outside or opposite side.

A particularly troublesome technical problem arises 40 when a high degree of hydrophobicity is desired in a nonwoven component produced substantially from conventionally bonded webs of hydrophobic fiber such as polyolefin-containing staple or spun-bonded webs.

In general, untreated hydrophobic fiber quickly 45 becomes unworkable due to friction and accumulated static charge generated during conventional spinning, cutting and carding operations. For this reason, the art has long recognized and used a variety of topically applied antistatic agents which change fiber surface 50 properties sufficiently to permit such conventional fiber processing. In effect, however, such treatment also produces fiber, web and nonwoven product which is substantially more hydrophilic than the untreated spun fiber.

Because of the nature of commercial high speed operations, and the somewhat unpredictable affinity of such agents to individual batches or bales of hydrophobic fiber, it becomes very difficult to maintain adequate control over bonding steps and over the wetting characteristics of the final nonwoven product.

It is an object of the present invention to prepare a hydrophobic polyolefin-containing spun fiber or filament for processing such as intermediate cutting and carding steps without unduly interfering with subsequent bonding steps or sacrificing needed hydrophobic characteristics in the nonwoven product.

**THE INVENTION**

The above objects are obtained in accordance with the present invention by preparing polyolefin containing spun fiber or filament in accordance with the steps of

- A. initially treating the corresponding continuous spun fiber or filament with an effective amount, varying from about 0.09%-0.5% based on fiber weight, of a first modifier composition comprising  
(a) about 70%-100% by weight of modifier composition of at least one neutralized phosphoric acid ester represented by the formula



wherein

Alk is individually defined as a lower alkyl group, such as a 1-8 carbon alkyl and preferably a 1-4 carbon alkyl group;

R is defined as an amino group or an alkali metal, n and m are individually defined as positive numbers of not less than about 1, the sum of which is about 3; and

- (b) up to about 30% by weight of modifier composition of at least one polysiloxane represented by the formula



wherein

X and Y are individually defined as a hydrophobic chemical end group such as a lower alkyl group; R' is individually defined as a lower alkyl such as a methyl group, and

o is defined as a positive number within the range of about 10-50 or higher;

- B. crimping the resulting continuous fiber or filament in a crimper;  
C. applying to said continuous fiber or filament preferably at a point proximate to said crimper an effective amount, varying from about 0.05%-0.20% by fiber weight, of a second modifier composition comprising  
(a) about 70%-100%, by weight of second modifier composition, of at least one polysiloxane represented by formula (2), and  
(b) up to about 30%, by weight of second modifier composition, of at least one neutralized phosphoric acid ester represented by formula (1);  
D. processing the resulting modifier-treated continuous fiber or filament, for spun bonding or for staple web bonding purposes, to obtain position one or more webs for bonding; and  
E. bonding the resulting web in a conventional manner to obtain a desired hydrophobic nonwoven material.
- For present purposes the term "polyolefin containing spun fiber or filament" includes continuous as well as staple melt spun fibers which are obtainable from conventionally blended isotactic polypropylene as well as art-recognized hydrophobic copolymers thereof with ethylene, 1-butene, 4 methylpentene-1 and the like. The resulting blended an extruded spun melt conveniently has a weight average varying from about  $3 \times 10^5$  to

about  $5 \times 10^5$ , a molecular weight distribution of about 5.0-8.0, a melt flow rate of about 2.5 to about 4.0 g/10 minutes, and a spin temperature conveniently within a range of about 220° C.-300° C.

Also includable within the spun melt are various art-recognized fiber additives, including pH stabilizers such as calcium stearate, antioxidants, pigments, including whiteners and colorants such as TiO<sub>2</sub> and the like. Generally such additives vary, in amount, from about 0.5%-3% by weight of spun melt.

The present invention is found particularly applicable to high speed production of a variety of nonwoven materials utilizing webs obtained, for instance, from spun bonded or carded staple and may also comprise additional web components such as fabricated film and the like. In each case, the fiber-handling difficulties generated by friction and accumulated static charge can be avoided, without unacceptable sacrifice in bonding characteristics (i.e. strength) or loss of hydrophobic properties of the final nonwoven product.

In this regard, the term "processing" as applied in process step "D" is inclusive of art recognized web formation techniques applicable to continuous as well as crimped, cut and carded staple fiber, the crimping step in the former case being optional with respect to webs formed solely of fiber or filament.

Continuous spun fiber or filaments used to form webs within the scope of the present invention preferably comprise topically treated spun melt staple fiber, filament or fibrillated film of bicomponent or monofilament types, the above-defined modifier compositions being conventionally drawn over a feed wheel partially immersed in a bath of the above defined modifier composition, dipped therein, or sprayed in effective amount for fiber processing, and dried.

For present purposes, webs used to form nonwovens within the scope of the present invention can be formed by spun bonded, melt blown or conventional "Dry" carded Process using staple fiber and bonded together using techniques employing adhesive binders (U.S. Pat. No. 4,535,013), calender rolls, hot air, sonic, laser, pressure bonding, needle punching and the like, known to the art.

webs used to fabricate nonwoven material can also usefully comprise conventional sheath/core or side-by-side bicomponent fiber or filament, alone or combined with treated or untreated homogeneous type fiber or filament and/or fibrillated film.

Also within the scope of the present invention is the use of nonwovens comprised of one or more bonded webs of modifier-treated polyolefin fiber and/or fiber-like (fibrillated film) components having a mixed fiber denier of homogeneous and/or bicomponent types not

exceeding about 40 dpf. Such webs preferably utilize fiber or filaments within a range of about 0.1-40 dpf.

In addition, the resulting nonwoven material can be embossed and/or calender printed conventionally with various designs and colors, as desired, to increase loft, augment wet strength, and provide easy market identification.

In addition, webs used in forming nonwovens within the scope of the present invention are produced from one or more types of conventionally spun fibers or filaments having, for instance, round, delta, trifocal, or diamond cross sectional configurations.

Nonwoven cover stock of the above defined types can usefully vary in weight from about 10-45 gm yd<sup>2</sup> or higher.

The invention is further illustrated but not limited by the following Examples and Tables:

#### EXAMPLE 1

20 A. Polypropylene in flake form and characterized as follows: (crystallinity 60% M<sub>w</sub>  $3.5 \times 10^5$ , molecular weight distribution 6.4, and melt flow 3.2 g/10 minutes) is mixed in an impact blender. After thorough blending, the mixture is fed into a 1 1/2" extruder and spun through 25 a 210 hole spinnerette at 280° C., air quenched, and stretched at 115° C. (4×) to obtain a 2 dpf circular filament which is then passed over a feed or kiss wheel partly immersed in a tank of first modifier composition consisting of a 50% aqueous solution of Lurol® AS-Y<sup>(1)</sup>, a neutralized phosphoric acid/alcohol ester, contact being of sufficient duration and speed to topically apply about 0.6 wt. % of the dried composition. The resulting continuous filament is crimped at about 30 100° C. and spray coated (0.10 wt %) with a second modifier composition consisting of a 20:1 mixture by weight of a 60% polydimethyl siloxane emulsion commercially available as LE-458HS<sup>(2)</sup> and a 50% aqueous solution of Lurol AS-Y. After air drying, the coated 2.0 dpf fiber is chopped to 1.5" length staple and set aside for conventional ASTM Sink Time tests in which a given weight of fiber is loosely packed into a mesh basket and the sink time measured in seconds. The remainder is carded into webs weighing about 20 g/yd<sup>2</sup>, two webs being calendar bonded at 162° C. to obtain 35 test nonwoven material. The test nonwoven is cut into strips of convenient dimensions for carrying out conventional strength and run off tests using syn urine<sup>(3)</sup> as the wetting fluid. Test results, are summarized and reported in Tables I and II.

<sup>(1)</sup>A product of George A. Goulet Company of Situate, Mass.

<sup>(2)</sup>A product of Union Carbide Corporation.

<sup>(3)</sup>Syn-urine is a product of Jayco Pharmaceuticals of Camp Hill, Pa.

TABLE I

| Sample #  | Color Type | Degree of Hydrophobicity <sup>*4</sup> | MFR  | STAPLE PROPERTIES |               |      | Tenacity gms | Elongation % | CPI  | Spin Fin. Type/AMT | Over Fin. Type/AMT     |
|-----------|------------|----------------------------------------|------|-------------------|---------------|------|--------------|--------------|------|--------------------|------------------------|
|           |            |                                        |      | Percent Tow       | Finish Staple | DPF  |              |              |      |                    |                        |
| S-1       | 195        | 5                                      | 17.6 | 0.77              | 0.41          | 2.6  | 2.05         | 308.7        | 28.9 | 263/0.6            | 262/0.3                |
| S-2       | 187        | 5                                      | 35.7 | 0.31              | 0.49          | 2.0  | —            | —            | —    | 263/0.2            | 262/0.3                |
| S-3       | 195        | 5                                      | 24.3 | 0.15              | —             | 2.2  | —            | —            | —    | 263/0.2            | 262/0.15 <sup>*5</sup> |
| S-4       | 187        | 5                                      | 21.7 | 0.48              | 0.48          | 2.43 | 1.68         | 402.0        | 25.1 | 263/0.2            | 262/0.3                |
| Lt. Blue  | 187        | 5                                      | 22.2 | 0.25              | 0.38          | 2.54 | 1.72         | 424.8        | 28.5 | 263/0.2            | 262/0.3                |
|           |            |                                        |      |                   |               |      |              |              |      |                    |                        |
| Med. Blue | 195        | 5                                      | 21.0 | 0.5               | 0.53          | 2.28 | 1.91         | 375.1        | 26.0 | 263/0.4            | 262/0.3                |
|           |            |                                        |      |                   |               |      |              |              |      |                    |                        |
| S-6       | 195        | 5                                      | 21.0 | 0.5               | 0.51          | 2.38 | 1.86         | 373.8        | 21.5 | 263/0.4            | 262/0.3 <sup>*6</sup>  |
| S-7       | 195        | 5                                      | 21.0 | 0.5               | 0.48          | 2.45 | 2.10         | 411.4        | 22.8 | 263/0.4            | 262/0.3 <sup>*7</sup>  |
| S-8       | 195        | 5                                      | 21.0 | 0.5               | 0.60          | 2.43 | 1.91         | 363.0        | 22.1 | 263/0.4            | 262/0.3 <sup>*8</sup>  |
| S-9       | 195        | 5                                      | 21.0 | 0.5               | 0.61          | 2.50 | 1.93         | 361.5        | 20.5 | 263/0.4            | 262/0.3 <sup>*9</sup>  |
| S-10      | 195        | 5                                      | 21.0 | 0.5               | —             | —    | —            | —            | 30.8 | 263/0.4            | 262/0.3                |
| S-11      | 187        | 5                                      | —    | 0.42              | —             | —    | —            | —            | —    | —                  | —                      |

TABLE I-continued

| Sample # | Color Type    | Degree of Hydrophobicity* <sup>4</sup> | MFR  | STAPLE PROPERTIES |               |      | Tenacity gms | Elongation % | CPI  | Spin Fin. Type/AMT | Over Fin. Type/AMT |
|----------|---------------|----------------------------------------|------|-------------------|---------------|------|--------------|--------------|------|--------------------|--------------------|
|          |               |                                        |      | Tow               | Finish Staple | DPF  |              |              |      |                    |                    |
| S-12     | Lt. Blue 187  | 5                                      |      | 0.45              | —             | —    | —            | —            | 30.8 | 263/0.4            | 262/0.3            |
| S-13     | Med. Blue 195 | 5                                      | 22.3 | 0.35              | 0.4           | 2.42 | 1.87         | 273.9        | 27.5 | 263/0.4            | 262/0.15           |
| S-14     | 187           | 5                                      | 19.8 | 0.47              | 0.52          | 2.36 |              |              | 21.3 | 263/0.4            | 262/0.3            |
| S-15     | Blue 187      | 5                                      | 20.9 | 0.56              | 0.53          | 2.42 | 1.80         | 297.0        | 27.8 | 263/0.4            | 262/0.3            |
| S-16     | Blue 225 187  | 5                                      | 20.8 | 0.44              | 0.48          | 2.13 | 1.92         | 347.0        | 26.3 | 263/0.4            | 262/0.3            |
|          | Blue 275      |                                        |      |                   |               |      |              |              |      |                    |                    |

\*<sup>4</sup>1 = Fully Hydrophilic; 5 = Fully Hydrophobic based on Fiber Sink Test.\*<sup>5</sup>Added Finish No. 262 to tow with kiss roll to reduce static. Total 262 add-on not known.\*<sup>6</sup>Finish No. 262 + 0.08 Lurol AS-Y;\*<sup>7</sup>Extra (0.24) Lurol AS-Y;\*<sup>8</sup>Extra 0.32 Lurol AS-Y;\*<sup>9</sup>Extra 0.72 Lurol AS-Y

TABLE II

## THERMOBONDED WEB

| Staple | Bond Temp., °C. | Bond Press. Pli | Line Speed ft./min. | *10 Strength, g/in. |     | *10 Elongation, % |     | Run-Off % | Rewet gms. | Strike Time sec. |
|--------|-----------------|-----------------|---------------------|---------------------|-----|-------------------|-----|-----------|------------|------------------|
|        |                 |                 |                     | MD                  | CD  | MD                | CD  |           |            |                  |
| S-1    | 165             | 160             | 250                 | 930                 | 271 | 43                | 86  | 98.3      | *11        | *11              |
| S-2    | 160             | 160             | 250                 | 892                 | 288 | 27                | 70  | 99.3      | *11        | *11              |
| S-3    | 157.5           | 160             | 100                 | 1294                | 325 | 30                | 77  | 97.3      | *11        | *11              |
| S-4    | 160             | 160             | 250                 | 1716                | 339 | 50                | 101 | 91.2      | *11        | *11              |
| S-5    | 155             | 160             | 100                 | 1500                | 423 | 37                | 87  | 94.7      | *11        | *11              |
| S-6    | 155             | 160             | 100                 | 1463                | 310 | 27                | 70  | 95.9      | 0.105      | *11              |
| S-7    | 155             | 160             | 100                 | 1345                | 292 | 27                | 76  | 95.0      | 0.120      | *11              |
| S-8    | 155             | 160             | 100                 | 1188                | 285 | 23                | 78  | 97.1      | 0.111      | *11              |
| S-9    | 155             | 160             | 100                 | 1325                | 255 | 28                | 70  | 94.1      | 0.102      | *11              |
| S-10   | 155             | 160             | 100                 | 1391                | 220 | 29                | 73  | 98.8      | 0.147      | *11              |
| S-11   | 152.5           | 160             | 100                 | 1244                | 257 | 31                | 71  | 93.0      | *11        | *11              |
| S-12   | 152.5           | 160             | 100                 | 1389                | 294 | 37                | 80  | 95.2      | *11        | *11              |
| S-13   | 150             | 160             | 100                 | *12                 | *12 | *12               | *12 | 91.5      | *11        | *11              |
| S-14   | 157.5           | 160             | 100                 | 1944                | 533 | 34                | 78  | 95.0      | *11        | *11              |
| S-15   | 157.5           | 160             | —                   | *12                 | *12 | *12               | *12 | 94.9      | *11        | *11              |
| S-16   | 157.5           | 160             | 100                 | 1347                | 392 | 26                | 80  | >90.0     | *11        | *11              |

\*<sup>10</sup> 20 g/yd<sup>2</sup> Web\*<sup>11</sup> Could not test. Solution remained on surface of fabric in Run Off Test (fully hydrophobic)\*<sup>12</sup> No determination run.

## I. claim:

1. A method for preparing essentially hydrophobic polyolefin-containing spun fiber or filament for cutting and carding steps in the production of hydrophobic nonwoven material, comprising

A. initially treating corresponding continuous spun fiber or filament with an effective amount of a first modifier composition comprising

(a) about 70%-100% by weight of modifier composition of at least one neutralized phosphoric acid ester represented by the formula



wherein

alk is individually defined as a lower alkyl group, R is defined as an amino group or an alkali metal, n and m are individually defined as positive numbers of not less than about 1, the sum of which is about 3; and

(b) up to about 30% by weight of modifier composition of at least one polysiloxane represented by the formula



(2)

wherein

X and Y are defined as hydrophobic chemical end groups,

R' is individually defined as a lower alkyl group, and

o is defined as a positive number within the range of about 10-50 or higher;

55 B. crimping the resulting continuous fiber or filament in a crimper;

C. applying to said fiber or filament an effective amount of a second modifier composition comprising

(a) about 70%-100%, by weight of second modifier composition, of at least one polysiloxane represented by formula (2), and

(b) up to about 30%, by weight of second modifier composition, of at least one neutralized phosphoric acid ester represented by formula (1);

60 D. processing the resulting modifier-treated fiber or filament to obtain one or more webs for bonding; and

E. bonding the resulting web to obtain a desired hydrophobic nonwoven material.

2. The method of claim 1 wherein initial treatment of said continuous spun fiber or filament is effected using about 100%, by weight of first modifier composition, of at least one neutralized phosphoric acid ester represented in formula (1).

3. The method of claim 1 wherein the Alk-O group of the neutralized ester is defined as a straight 1-4 carbon alkoxy group; n is 2; and m is 1.

4. The method of claim 1 wherein the second modifier composition is topically applied upstream of said crimper.

5. The method of claim 1 wherein the second modifier composition is topically applied to an at least partially crimped continuous spun fiber or filament.

6. The method of claim 1 wherein the "D" processing step comprises a fiber cutting and carding operation.

7. The method of claim 1 wherein the "D" and "E" steps comprise a spun bonding operation.

8. A Crimped essentially hydrophobic polyolefin-containing fiber obtained by

A. initially treating corresponding continuous spun fiber or filament with an effective amount of a first modifier composition comprising

(a) about 70%-100% by weight of modifier composition of at least one neutralized phosphoric acid ester represented by the formula



wherein

Alk is individually defined as a lower alkyl group, R is defined as an amino group or an alkali metal, n and m are individually defined as positive numbers of not less than about 1, the sum of which is about 3; and

(b) up to about 30% by weight of modifier composition of at least one polysiloxane represented by the formula

50



wherein X and Y are defined as hydrophobic chemical end groups,

R' is individually defined as a lower alkyl group, and

o is defined as a positive number within the range of about 10-50 or higher;

B. crimping and applying to said fiber or filament an effective amount of a second modifier composition comprising

(a) about 70%-100%, by weight of second modifier composition, of at least one polysiloxane represented by formula (2), and

(b) up to about 30%, by weight of second modifier composition, of at least one neutralized phosphoric acid ester represented by formula (1).

9. The fiber of claim 8 wherein initial treatment of said continuous spun fiber or filament is effected using about 100%, by weight of first modifier composition, of at least one neutralized phosphoric acid ester represented in formula (1).

10. The fiber of claim 8 wherein the Alk-O group of the neutralized ester is defined as a straight 1-4 carbon alkoxy group; n is 2; and m is 1.

11. The fiber of claim 10 wherein the second modifier composition is topically applied upstream of said crimper.

12. The fiber of claim 9 wherein the second modifier composition is topically applied to an at least partially crimped continuous spun fiber or filament.

13. A nonwoven material obtained in accordance with claim 1.

14. A nonwoven material obtained in accordance with claim 2.

15. A nonwoven material obtained in accordance with claim 3.

16. A nonwoven material obtained in accordance with claim 4.

17. A nonwoven material obtained in accordance with claim 5.

18. A nonwoven material obtained in accordance with claim 6.

19. A nonwoven material obtained in accordance with claim 7.

\* \* \* \* \*

UNITED STATES PATENT AND TRADEMARK OFFICE  
CERTIFICATE OF CORRECTION

PATENT NO. : 4,938,832

Page 1 of 3

DATED : July 3, 1990

INVENTOR(S) : SCHMALZ

It is certified that error appears in the above-identified patent and that said Letters Patent is hereby corrected as shown below:

Column 1, Lines 8 and 9, " polyolefin containing "  
should read -- polyolefin-containing --

Column 1, Line 15, " polyolefin based "  
should read -- polyolefin-based --

Column 1, Line 23, " fluid absorbent "  
should read -- fluid-absorbent --

Column 1, Line 28, " fluid absorbing "  
should read -- fluid-absorbing --

Column 1, Line 44, " staple "  
should read -- staple- --

Column 2, Lines 5 and 6, " polyolefin containing "  
should read -- polyolefin-containing --

UNITED STATES PATENT AND TRADEMARK OFFICE  
CERTIFICATE OF CORRECTION

PATENT NO. : 4,938,832

Page 2 of 3

DATED : July 3, 1990

INVENTOR(S) : SCHMALZ

It is certified that error appears in the above-identified patent and that said Letters Patent is hereby corrected as shown below:

Column 2, Lines 61 and 62,

" "polyolefin containing spun fiber or filament" "

should read

-- "polyolefin-containing spun fiber or filament" --

Column 2, Line 66, " 4 methylpentene-1 "

should read -- 4-methylpentene-1 --

Column 2, Line 67, " an "

should read -- and --

Column 3, Line 15, " fabricated "

should read -- fibrillated --

Column 3, Line 33, " above defined "

should read -- above-defined --

UNITED STATES PATENT AND TRADEMARK OFFICE  
CERTIFICATE OF CORRECTION

PATENT NO. : 4,938,832

Page 3 of 3

DATED : July 3, 1990

INVENTOR(S) : SCHMALZ

It is certified that error appears in the above-identified patent and that said Letters Patent is hereby corrected as shown below:

Column 4, Line 11, " trifocal, "

should read -- trilobal, --

Column 5, Claim 1, Line 61, " alk "

should read -- Alk --

Column 6, Claim 1, Line 59, " (as) "

should read -- (a) --

Column 7, Claim 8, Line 24, " Crimped "

should read -- crimped --

Signed and Sealed this

Seventeenth Day of December, 1991

*Attest:*

HARRY F. MANBECK, JR.

*Attesting Officer*

*Commissioner of Patents and Trademarks*